

## UNITED STATES PATENT OFFICE

2,185,453

METHOD OF HEAT TREATING MAGNESIUM  
BASE ALLOYSRobert T. Wood, Cleveland, Ohio, assignor, by  
mesne assignments, to Magnesium Develop-  
ment Corporation, a corporation of DelawareNo Drawing. Application September 1, 1937,  
Serial No. 161,948

5 Claims. (Cl. 148—21.3)

This invention relates to magnesium base alloys and it is especially concerned with accelerating the heat treatment of certain cast alloys.

Magnesium base alloys which contain aluminum and zinc as the chief added alloying ingredients have been used for some time in the production of castings because of their good casting characteristics and relatively high strength as compared to other magnesium base alloys.

Although castings of these alloys are suitable for many purposes in the as-cast form yet it has been found that their strength can be materially increased by subjecting them to a solution heat treatment followed by rapid cooling to room temperature. It ordinarily requires a heating period lasting for a number of hours to secure the desired degree of solution of the soluble constituents in the cast alloys. In some instances, as for example in the case of cast magnesium base alloys of the type containing from 1 to 12 per cent aluminum, and 0.3 to 5 per cent zinc, it has been found to be necessary to employ a two-step thermal treatment consisting of an initial heating at about 630° F. for several hours followed by heating at about 720° F. for a longer period of time, to obtain the desired degree of solution of the alloy ingredients. Exposure of the castings to higher temperatures for a shorter period of time as a means of reducing the time of heat treatment has been considered to be impractical because of the danger of intergranular melting and oxidation with consequent reduction in the mechanical properties of the casting.

It is an object of my invention to provide a means of hastening the solution heat treatment of cast magnesium base alloys containing from 1 to 12 per cent aluminum and 0.3 to 5 per cent zinc. Another object is to avoid the necessity for using the two-step thermal treatment which has heretofore been the standard practice in treating castings of this type. Still another object is to obtain substantially the same strength in solution heat treated cast magnesium base alloys containing aluminum and zinc in a much shorter time than has been considered possible heretofore.

My invention is based upon the discovery that the addition of from about 0.03 to 0.3 per cent calcium to cast magnesium base alloys containing from about 1 to 12 per cent aluminum and 0.3 to 5 per cent zinc permits a more rapid solution heat treatment of the castings at a higher temperature than has hitherto been regarded as being a safe practice. In the case of castings

containing calcium it is necessary to use only one solution heat treatment instead of the customary two-step process. Furthermore, it has been found that neither the presence of calcium nor the shorter heat treatment reduces the strength of the castings as compared to similar castings containing no calcium and treated by the two-step method.

Although the addition of calcium is beneficial to alloys containing aluminum and zinc in the amounts mentioned above, it is especially advantageous in alloys containing from 4 to 8 per cent aluminum and 2 to 4 per cent zinc. It is also my preferred practice to add from 0.03 to 0.1 per cent calcium to these alloys as well as those containing larger amounts of aluminum and zinc. Some alloy compositions that are particularly recommended for the production of heat treated castings contain 6 per cent aluminum, 3 per cent zinc and 0.05 per cent calcium; 10 per cent aluminum, 1 per cent zinc and 0.05 per cent calcium.

The alloys may be made in the usual manner through the use of rich alloy hardener or by the addition of the pure metal. The alloys should be melted and cast under the conditions usually prevailing in magnesium alloy foundries, that is, the melt should be protected against oxidation and the sand molds should be treated to prevent a burning of the metal. The alloys may be cast within the customary range of pouring temperatures.

The castings should be heat treated by subjecting them to a temperature of 720 to 780° F. for a period of 5 to 30 hours, followed by a rapid cooling to below 400° F., generally to room temperature. If desired they may be artificially aged in the usual manner after the foregoing thermal treatment. In my preferred practice the castings are heated at 750° F. for 10 hours and then rapidly cooled to room temperature. I have found that it is necessary to heat alloys of the foregoing type to at least 720° F. to secure a solution of the soluble constituents within a reasonable length of time. At temperatures above 780° F., however, there is danger of incipient melting and/or intergranular oxidation with a consequent weakening of the cast article. As to the length of time required for heating the castings, it has been my experience that at least 5 hours is needed to obtain a substantial degree of solution and that a complete solution is obtained within 30 hours.

Although the presence of 0.03 to 0.3 per cent calcium is useful in reducing the time required

for heat treatment of the cast alloys by reason of the fact that higher temperatures can be employed, yet in greater concentrations than 0.3 per cent this element hinders or may even prevent the solution of the  $Mg_3Al_2$  constituent in the alloy. I have observed, for example, if more than 0.3 per cent calcium is present that the solubility of the intermetallic compound,  $Mg_3Al_2$ , is so reduced that a satisfactory solution and increase in strength of the alloy can not be obtained within a reasonable time even at a heat treating temperature as high as 810° F. On the other hand, less than 0.03 per cent of this element has no substantial effect upon the solubility of the aforesaid compound, and it also is ineffective as far as decreasing the time required for heat treating the alloy is concerned. In the range between 0.03 and 0.3 per cent, however, there is an effect upon the solubility of the  $Mg_3Al_2$  compound but it is subordinate to the advantage gained in reducing the time required for the solution heat treatment. In other words, the increase in the rate of solution gained by using a higher heat treating temperature than has been heretofore employed in commercial practice more than offsets the solution impeding effect of 0.03 to 0.3 per cent calcium.

Having thus described my invention and certain embodiments thereof, I claim:

1. A method of producing, in a heat-treated magnesium base alloy containing 1 to 12% aluminum and 0.3 to 5% zinc, properties commensurate with those obtained by a two-step solution heat treatment, the method comprising adding 0.03 to 0.3% calcium to said alloy, casting the resulting alloy, subjecting the resulting casting to a single step solution heat treatment at a temperature between 720 and 780° F., and rapidly cooling said heat-treated casting to a temperature below 400° F.

2. A method of producing in a heat-treated magnesium base alloy containing 1 to 12% alumi-

num and 0.3 to 5% zinc, properties commensurate with those obtained by a two-step solution heat treatment, the method comprising adding 0.03 to 0.3% calcium to said alloy, casting the resulting alloy, subjecting the resulting casting to a single step solution heat treatment at a temperature between 720 and 780° F. for 5 to 30 hours, and rapidly cooling said heat-treated casting to a temperature below 400° F.

3. A method of producing in a heat-treated magnesium base alloy containing from 4 to 8% aluminum and 2 to 4% zinc, properties commensurate with those obtained by a two-step solution heat treatment, the method comprising adding 0.03 to 0.1% calcium to said alloy, casting the resulting alloy, subjecting the resulting casting to a single step solution heat treatment at a temperature between 720 and 780° F. for 5 to 30 hours, and rapidly cooling said heat-treated casting to a temperature below 400° F.

4. A method of producing, in a casting of a magnesium base alloy containing 1 to 12% aluminum, 0.3 to 5% zinc, and 0.03 to 0.3% calcium, properties commensurate with those obtained by a two-step solution heat treatment, the method comprising subjecting the casting to a single step solution heat treatment at a temperature between 720 and 780° F. for 5 to 30 hours, and rapidly cooling said heat-treated casting to a temperature below 400° F.

5. A method of producing, in a casting of a magnesium base alloy containing from 4 to 8% aluminum, 2 to 4% zinc, and 0.03 to 0.1% calcium, properties commensurate with those obtained by a two-step solution heat treatment, the method comprising subjecting the casting to a single step solution heat treatment at a temperature between 720 and 780° F. for 5 to 30 hours, and rapidly cooling said heat treated casting to a temperature below 400° F.

ROBERT T. WOOD.